

Aug. 25, 1959

R. B. POND

2,900,708

APPARATUS FOR PRODUCING ALLOY AND BIMETALLIC FILAMENTS

Filed Feb. 16, 1956



Fig. 1

Fig. 2



Fig. 5



Fig. 6



Fig. 7



Fig. 8

Fig. 10



Fig. 3



Fig. 9



Fig. 4

1

2,900,708

**APPARATUS FOR PRODUCING ALLOY AND BIMETALLIC FILAMENTS**

Robert B. Pond, Westminster, Md., assignor to Marvalaud, Incorporated, Westminster, Md., a corporation of Maryland

Application February 16, 1956, Serial No. 565,814

4 Claims. (Cl. 29—194)

This invention relates to a method of producing metal fibers and filaments and, more particularly, to the production of anisotropic filaments.

Anisotropic bodies, such as bimetallic filaments, wires and like bodies are generally formed by welding or cladding metals whereby the metals at their adjacent surfaces are brought to a sufficiently high temperature either with or without applied pressure to produce an interdiffusion of one metal into the surface of the other metal. The bond thus formed is sufficient to form a unitary body. Wires or filaments formed of an alloy, on the other hand, have a substantially uniform composition laterally across the body.

The term "filament" is used herein and in the claims to designate bodies or elements having a relatively great or indefinite length with respect to their transverse sectional dimensions.

One of the purposes of the present invention is to provide a method for the production of anisotropic metallic filaments.

Another object of this invention is to provide a method for the production of bimetallic filaments.

A further object of this invention is to provide metallic alloy filaments wherein the composition of the filaments varies transversely across the filaments.

Other objects and advantages of this invention will become apparent from the description and claims which follow.

In the accompanying drawings:

Figure 1 is a cross-sectional view of an ejector tube adapted for the practice of this invention;

Figure 2 is a cross-sectional view of a further embodiment of an ejector tube for the practice of this invention;

Figure 3 is a perspective diagrammatic view showing one form of means for forming metal filaments;

Figure 4 is a sectional diagrammatic view showing another embodiment of apparatus for forming filaments in accordance with this invention;

Figures 5, 6, 7, 8 and 9 are diagrammatic cross-sectional views of products formed in accordance with the present invention; and

Figure 10 is a cross-sectional view of another form of ejector tube.

The method of the present invention contemplates joining or bringing together two or more streams of molten metals to form a single stream of molten metal and converting the stream into solid filaments. The present invention further contemplates an extrusion nozzle having separate ducts or channels for different metals, the ducts being so arranged as to bring together the streams of molten metal.

One embodiment of the products of this invention consist of filaments formed of two different metals which alloy with each other wherein the composition varies progressively in a direction transverse to the filament. In a second embodiment, the filaments comprise two sepa-

rate metals which do not alloy with each other but interdiffuse and adhere to each other.

As illustrated in Figure 1, there is provided a suitable ejector tube or cylinder 1 including a partition 2 adapted to contain the molten metals A and B and from which the molten metals are extruded under pressure. The chamber may be in the nature of a crucible having heating means and the metals may be melted within the crucible or the molten metals may be supplied from crucibles 10 3 and 4. An extrusion die 5 formed of a suitable ceramic or other refractory material is removably mounted at one end of the chamber 1. The die is provided with extrusion ducts or orifices 6 and 7 each of which communicates with one of the chambers within the cylinder. The extrusion ducts may be of any desired size and are arranged at an angle so as to direct the streams of molten metal toward each other. The opposite end of the cylinder 1 is closed by means of a removably mounted plate which is provided with gas ducts 8 and 9 which communicate 15 with a source of gas under pressure. In the operation of the device, the molten metals are extruded by supplying gas under pressure. The streams of metal are joined or brought together while both metals are in a molten state.

The apparatus as shown in Figure 2 includes a like ejector tube or crucible 10 having a movable partition 11. The separate chambers may be supplied with molten metals A and B as described. The extrusion die 12 having an extrusion duct or orifice 13 communicates with the chambers of the cylinder through a conical throat 14. 20 A truncated conical plug 15 is secured at the lower end of the partition 11 and is so arranged to extend into the throat 14 in the die. In order to provide a continuous stream of molten metal, the metals are extruded under pressure which may be supplied by a gas supplied to the conduits 16 and 17 in the closure for the cylinder. The molten metals thus flow from their respective chambers toward the extrusion orifice 13 through the ducts or channels formed between the throat 14 and the plug 15 and the molten metals are joined or brought together as they 25 approach the extrusion orifice.

If it is assumed that the orifices 6 and 7 in the die 5 (Figure 1) are of the same size and if it is assumed that the partition 11 and plug 15 (Figure 2) are centrally disposed with respect to the die 12, equal volumes of the two metals will be brought together to form a continuous stream of molten metal. The stream of molten metal as provided by the apparatus of Figure 1 or Figure 2 may be converted into a solid filament by the method as disclosed in my copending application Serial No. 387,187, 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 946

In my copending applications Serial No. 563,541 and Serial No. 563,615, both filed February 6, 1956, there are disclosed methods and apparatus for transforming continuous streams of molten metal into filaments of any desired cross-sectional configuration from non-refractory metals. The apparatus of these applications are illustrated diagrammatically in Figure 4. The extrusion apparatus of the present invention may be utilized in this method and apparatus to form the filaments of two or more metals.

The ejector tube 22 is positioned at the top of a suitable tower 23 at the bottom of which there is disposed a suitable collecting box or truck 24. Gas conduits 25 and 26 communicate with the interior of the tower at the bottom and top, respectively. For metals which do not readily oxidize in air such as lead and tin, for example, the molten metal may be extruded in air. For metals which oxidize readily in air, the tower may be supplied with an inert gas such as nitrogen, helium or the like through conduits 25 and 26. Where the gas is heavier than air, the gas may be supplied to the tower through conduit 25 whereby the air is flushed from the tower at the top through conduit 26. For gases lighter than air, the gas is supplied at the top of the tower through conduit 26 and the air flushed from the tower through conduit 25. In those instances where the metal has a high vapor pressure at the extrusion temperatures, the gas within the tower may be maintained under sufficient pressure to overcome the vapor pressure of the metal. In all instances, the pressure within the ejector tube 22 must be regulated to provide a continuous stream of molten metal leaving the extrusion cylinder and where the gas within the tower is maintained under pressure, the pressure in the ejector tube 22 must, of course, be greater than the pressure within the tower. For example, where one of the metals being extruded is zinc, the gauge pressure within the tower may be maintained at about ten pounds per square inch.

In one embodiment where the two metals readily alloy with each other, for example, if the metal A is lead and the metal B is tin, the resulting filament will consist of an alloy. In view of the fact that the molten metals solidify in a very brief period of time, the composition will not be uniform transversely of the filament. If it is further assumed for purposes of illustration that a round filament is formed as shown in Figure 5 by utilizing the apparatus of Figure 4, the composition on one side of the filament will be substantially entirely metal A or lead and on the other side the filament will be substantially all metal B or tin. The relative proportions of metals A and B in the alloy vary progressively across the filament because the time in which the two metals are in contact in molten condition with each other is not sufficient to permit a thorough solution of one metal throughout the other metal. It will be understood, however, that where the combined stream of molten metals is very small, the product may not have edges or sides consisting of substantially pure metal but may consist of an alloy where the edges or sides are rich on one of the metals.

In another embodiment where the two metals do not readily alloy with each other but adhere to each other, the product will be a bimetallic filament as illustrated diagrammatically in Figure 6. One portion of the wire will consist of metal A and the other portion will consist of the metal B separated by an alloy zone or a boundary layer where there has been a slight diffusion of one metal into the other as indicated by the broken line 27.

In transforming the molten metal stream into the solid fiber by the use of apparatus as illustrated in Figure 3, the filament 21 has a more or less rectangular cross-section. The foregoing discussion with respect to the composition and structure of the filaments also applies to such "rectangular" filaments. It is obvious that the variation of composition of these "rectangular" filaments

may be varied depending upon the relative positions of the metals A and B as the combined molten metal stream impinges on the rotating chill block. Where, for example, the ejector tube is so positioned that the chamber containing one metal is above the chamber containing the other metal, the composition will vary across the minor cross-sectional axis of the filament. Thus, if the two metals do not alloy with each other and the chamber containing metal B is above the chamber containing metal A, the top portion of the filament would consist of metal B and the bottom portion consist of metal A. Where the ejector tube is so arranged that the chambers containing the two different metals are side-by-side in a horizontal direction, the filament would have the variation in composition along its major cross-sectional axis.

The foregoing discussion has been based upon an assumption that the extrusion orifices 6 and 7 (Figure 1) are of equal cross-sectional area and that the plug 15 (Figure 2) is centrally positioned within the throat of the extrusion nozzle 12. Anisotropic or bimetallic elements consisting of a major proportion of one metal may be formed by varying the relative volumes of the metals which are extruded. For example, a product consisting of a major portion of metal B and a minor or skin portion on one side of the metal A as illustrated diagrammatically in Figure 7 may be formed by providing the extrusion nozzle 5 with an orifice 6 which is relatively small with respect to the extrusion nozzle 7 or by moving the plug 15 to the left side of the extrusion nozzle 12 of Figure 2. If the orifice 7 in extrusion nozzle 5 is of relatively small cross-section with respect to orifice 6 or if the plug 15 is moved to the right side of the nozzle 12, the product would be as represented by Figure 8 wherein the metal A constitutes the major portion of the filament and metal B, the minor portion. Where the metals do not alloy with each other but merely interdiffuse to bond them together, the individual metals are separated by a boundary layer 27 as described hereinbefore.

These embodiments may be illustrated specifically, merely for the purposes of illustration, by reference to the production of filaments of lead and tin. The extrusion temperature may, for example, be about 350° C. which is roughly 20° above the melting point of lead and about 120° above the melting point of tin. Where the apparatus of Figure 2 is employed to form the continuous stream of molten metal, the temperature must necessarily be above the melting point of the lowest melting metal. In the use of apparatus as shown in Figure 1, partition 2 may be formed of a suitable refractory and insulating material so that the temperature of the lowest melting metal need not be about the same as that of the higher melting point metal. It is, however, necessary that the temperature of both metals be such that the streams of metal when they contact each other or become joined are both in molten state. The extrusion orifices 6 and 7 in the case of the apparatus of Figure 1 may be of a diameter of about 1.5 mils. For the apparatus as shown in Figure 2, the extrusion orifice may be about 2 mils in diameter. The pressure applied to the surfaces of the molten metals within the ejector tube may be in the neighborhood of about six pounds to about ten pounds per square inch (gauge) so as to form the continuous stream of molten metal. The rotating chill block may be formed of aluminum and may be about three inches in diameter. The chill or upper surface has a radius of curvature of about five inches and the angle at which the stream of molten metal impinges on the chill block may be about 30°. The resulting filament is a ribbon-like filament which may vary in thickness and width depending upon the velocity of the rotating chill block. At impingement velocities of 2 to 300 feet per second, the thickness is of the order of about 0.2 mil to about 0.4 mil and the width from about 15 to about 38 mils. The thickness may be decreased and the width increased by increasing the velocity of the

chill block or the thickness may be increased and the width decreased by reducing the velocity of the chill block.

Although the invention is illustrated specifically by reference to the production of lead-tin alloy filaments formed by the use of apparatus shown in Figure 3, the invention is not restricted to such products and apparatus or method. The lead-tin filaments also may be formed by the use of any other suitable apparatus such as that shown in Figure 4. Filaments may be formed in like manner of other alloys such, for example, as copper-nickel alloys, aluminum-zinc alloys and the like. Bimetallic filaments may be formed in like manner as described hereinbefore from combinations of metals such, for example, as copper-iron, aluminum-copper, aluminum-nickel, zinc-tin and the like. Where the alloys or one or both of the metals oxidize readily in air at the required extrusion or ejection temperature, the filaments are produced by the use of an inert atmosphere in apparatus of the type shown in Figure 4. Where one or both of the metals has a high vapor pressure at the required extrusion or ejection temperature, for example, in producing copper-zinc filaments, the filaments are produced by the use of apparatus as illustrated in Figure 4 and the gas in the tower or chamber is maintained under a pressure at least as high as the vapor pressure of the metal at the extrusion temperature.

In a further embodiment as illustrated diagrammatically in Figure 9, the composition of the filament varies radially along a transverse section of the filament; that is, the filament has a core 28 surrounded by a sheath 29. Where the metals do not alloy with each other, the metals will be separated by a boundary layer 30. In those instances where the metals alloy with each other, the center of the core may be composed entirely of one metal and the outer surface of the sheath composed of the other metal with progressively changing proportions of the two metals along the radius.

A further embodiment of apparatus of this invention particularly adapted for the production of filaments of this type is shown in Figure 10. The ejector tube or cylinder 31 comprises an outer crucible 32 and an inner crucible 33 mounted concentrically with respect to each other. The outer crucible is provided with a conical exit port 34 at one end and a closure at its other end. The inner crucible is formed with a closure at its upper end and a conical terminal end 35 having the desired size extrusion orifice. The slope or angle of the terminal end may be substantially the same as the slope of the exit port 34 so that the extrusion orifices for the two metals are at an acute angle with respect to each other. The inner crucible is preferably so arranged that it may be moved axially with respect to the outer crucible, thereby permitting a convenient means for regulating the thickness of the sheath. Suitable conduits are provided to introduce molten metal and to supply a gas under pressure to the crucibles as described hereinbefore. The operation of the apparatus is similar to that of the device illustrated in Figure 2. The molten metals are continuously extruded by the pressure of the gas and brought together as they emerge from the extrusion orifices. The thickness of the sheath may be varied by altering the relative positions of the crucible which, of course, alters the width of the annular orifice between the port 34 of the outer crucible and the conical end 35 of the inner crucible.

In the production of filaments by the use of this embodiment of the apparatus, the same factors must be considered as in the use of the previous described embodiments. For example, in forming tin-lead filaments, the temperatures, pressures and other factors may be as described hereinbefore. The ejector tube may be utilized with a tower as illustrated in Figure 4 and the atmosphere and pressure of the atmosphere in the tower are maintained to meet the requirements of the particular

metals. Filaments may be formed from other metals which alloy with each other, for example, copper and nickel, aluminum and zinc, copper and silver, etc. Bimetallic filaments or clad filaments may be formed of metals which do not alloy with each other, for example, aluminum-uranium, copper-iron, aluminum-copper, aluminum-nickel, zinc-tin, etc. Where one or both of the metals has a high vapor pressure at the particular temperatures involved in the extrusion, for example, in forming an aluminum clad uranium filament, the apparatus of Figure 4 is utilized and the atmosphere in the tower is maintained sufficiently high to prevent vaporization or volatilization of the metal of high vapor pressure, aluminum in this specific instance. If it is desired, for example, to completely sheath one metal such as uranium with another metal such as aluminum, the flow of the metal forming the sheath is first initiated and then the core metal extruded. In terminating the filament, the extrusion of the core metal is first arrested and finally the flow of the sheath metal is arrested.

It is well known that alloy wire or filament has a uniform composition in a direction transverse of the wire or filament. This invention provides for the first time alloy filaments or wire where the composition is not uniform but varies progressively across the filament as described hereinbefore.

The products of this invention differ completely in crystal or grain structure as compared to prior art products in that there has been no deformation of the crystals. The rapid chilling and solidification produces a cast structure while in prior art products the grains or crystals are elongated because of the mechanical working of the metal in producing wire or sheet forms. In the case of the bimetallic filaments of this invention, the chemical composition of the filaments may be substantially the same as that of bimetallic products produced by conventional methods. However, the grain or crystal structures of the products of this invention and the conventional methods differ completely as described with respect to alloy products.

As pointed out in detail in my copending application Serial No. 387,187, filed October 20, 1953, and when utilizing the chill plate, the cast metal filaments are solidified in a rectilinear shape with only one mold wall, namely, the smooth polished open surface of the chill block. Actually, the top and bottom surfaces of the cast metal ribbon-type filaments formed are separately and clearly identifiable, only the bottom surface bearing any indications of having engaged a mold surface. The upper surface of the filaments is characterized by shrinkage marks, relief dendrites, and line striae or mammiforms, whereas the bottom surface which has engaged the chill block is smooth with the exception of polishing pit marks, buffing marks, and the imprint caused by any engraving or the like on the block.

Cast filaments may be formed at solidification rates of from 50 to 1000 feet per second. As will be appreciated from the foregoing description these rates may be controllably varied to effect various desired results.

In view of the great speed of solidification effected, it is pertinent to note the method of measuring the solidification rate. The cast filaments formed carry on their bottom surfaces the impression of any mark placed on the chill surface. Since the surface tension of all molten metals is high it is obvious that the metal must have solidified while on the chill surface. The metal is never on the chill surface for one complete revolution of the surface (for if it was it would result in overlay or piling up of the material). In fact, with the present invention as described, only about one-half inch of the filament contacts the surface at any one time, that is to say, the molten metal goes onto the surface of the chill block at the same rate that the solid cast metal comes off. Then, since it is transformed from a liquid to a solid while on the rotating chill block, its minimum velocity of solidi-

fication can be calculated knowing the speed of the surface at the point of impingement and the length of filament making contact at any one time.

The foregoing description and specific examples are not intended as limitations of the invention but are to be considered as being illustrative. It is apparent that various changes and modifications may be made without departing from the spirit and scope of the invention.

I claim:

1. An article of manufacture comprising a cast metallic anisotropic filament formed of at least two metals substantially simultaneously solidified wherein the composition varies continuously and progressively throughout the transverse direction of the filament from substantially 100% of one metal on one side of the filament to substantially 100% of the other metal on the other side of the filament.

2. In a method for producing filaments formed of at least two metals comprising the steps of continuously extruding each of the metals in a molten state to form 20 streams of molten metals, bringing the streams of molten metals together to form a continuous, single stream of molten metal and thereafter solidifying the stream of molten metal into a filament having a composition varying in the transverse direction of the filament from substantially 100% of one metal on one side to substantially 100% of the other metal on the other side of the filament.

3. In a method according to claim 2 including the step of bringing the metals in a molten state together to form a continuous single stream of molten metal through 30 a gaseous cooling medium maintained under pressure until the stream has solidified into a filament.

4. The method for producing filaments formed of at

least two metals which comprises bringing the metals in a molten state together to form a continuous single stream of molten metal, impinging the continuous single stream of molten metal against a concave chill surface, rotating the concave chill surface on an axis coincident with the center of concavity of the surface so that the surface moves relative to the stream of metal as it impinges upon the moving surface, solidifying the stream of molten metal on the chill surface so as to form a filament having a composition varying continuously and progressively throughout the transverse direction thereof.

#### References Cited in the file of this patent

#### UNITED STATES PATENTS

|           |                 |                |
|-----------|-----------------|----------------|
| 87,862    | McClosky        | Mar. 16, 1869  |
| 279,346   | Cookson         | June 12, 1883  |
| 745,786   | Cole            | Dec. 1, 1903   |
| 989,075   | Staples         | Apr. 11, 1911  |
| 1,192,467 | Scott           | July 25, 1916  |
| 2,128,941 | Hudson          | Sept. 6, 1938  |
| 2,129,703 | Merle           | Sept. 13, 1938 |
| 2,181,987 | Beaver et al.   | Dec. 5, 1939   |
| 2,543,936 | Reynolds        | Mar. 6, 1951   |
| 2,569,150 | Brennan         | Sept. 25, 1951 |
| 2,586,046 | Huebner         | Feb. 19, 1952  |
| 2,598,344 | Brennan         | May 27, 1952   |
| 2,611,163 | Schaefer et al. | Sept. 23, 1952 |
| 2,683,676 | Little et al.   | July 13, 1954  |

#### FOREIGN PATENTS

|         |               |                |
|---------|---------------|----------------|
| 4,391   | Great Britain | Sept. 15, 1882 |
| 46,293  | Germany       | Feb. 10, 1911  |
| 844,806 | Germany       | July 24, 1952  |